

Oct. 13, 1959

H. G. LAUTERBACH ET AL

2,908,064

NON-WOVEN FILAMENTARY PRODUCTS AND PROCESS

Filed Oct. 31, 1956

*Fig. 1*



*Fig. 2*



*Fig. 3*



*Fig. 4*



*Fig. 5*



INVENTORS  
HERBERT G. LAUTERBACH  
HARRY M. NORTON

BY *Raymond E. Blumenthal*

ATTORNEY

1

2,908,064

## NON-WOVEN FILAMENTARY PRODUCTS AND PROCESS

Herbert G. Lauterbach and Harry M. Norton, Wilmington, Del., assignors to E. I. du Pont de Nemours and Company, Wilmington, Del., a corporation of Delaware

Application October 31, 1956, Serial No. 619,469

18 Claims. (Cl. 28—72)

This invention relates to formation of continuous filamentary material into non-woven coherent pliable felt-like articles.

Felting of wool and fur represents the oldest method of forming textile fabric. Conversion of continuous filaments into a coherent felt-like article cannot be accomplished by the usual felting process, which requires preliminary compaction or "hardening" followed by mechanical working with addition of heat and usually moisture. Felting appears to be dependent upon interlacing and intertwining of the fiber lengths; hence, the recognized unsuitability of continuous filaments for similar processing, although relatively stiff and brittle articles can be formed from batts of continuous filaments by bonding of the filaments, as by fusion or use of an adhesive.

It is also known that acrylonitrile polymer fibers do not felt well even in wool blends because of their stiffness. To prepare a good felt from acrylonitrile polymers or copolymers in blends with wool (50/50 or higher proportions of acrylonitrile polymer fiber) it is necessary to treat the blends with about 10% aqueous sodium thiocyanate solution at about 90° C. before felting.

One object of this invention is to provide a non-woven coherent pliable unbounded (i.e., unbounded and unadhered) felt-like article comprising predominantly synthetic organic continuous filamentary material, said article being characterized by predominantly coplanar orientation of the filamentary components in superimposed layers with portions of some of the filamentary components from each layer oriented into at least one adjacent layer.

Another object of this invention is to provide a non-woven coherent pliable felt-like article comprising retractable predominantly synthetic organic continuous filamentary material; also, the retracted article obtainable therefrom.

Another object of this invention is to provide processes for producing the above-described articles.

Other objects of this invention, together with means and methods for obtaining them, will be apparent from the following description and the accompanying diagrams.

The felt-like articles of this invention resemble wool felts except for the different structure of the article and composition and character of the filamentary material. The structure may be distinguished by the presence of superimposed layers of a preponderance of synthetic organic continuous filamentary material, portions of which are oriented into at least one adjacent layer of filamentary material, that is, portions of some of the filamentary material are oriented in the thickness direction of the felt-like article. The oriented filamentary material does not detract from the utility of the felt-like article but actually substantially reinforces the article and particularly so because the filamentary material is unfused and unbonded and each filament is free to move over adjacent filaments, thereby imparting great flexibility to the

2

article. The felt-like articles of this invention are easily distinguished from felted products containing thermoplastic fibers which have been bonded together by coating or impregnating with resins or heated until many of the filaments are fused together. In bonded articles of this sort the adhered fibers are not free to move relative to one another, and these resin-treated or heat-bonded products are stiff and undesirable for many applications where the strong pliable long-wearing felts of this invention may be used to advantage.

The invention will be understood more readily by reference to the drawings.

Figure 1 is a schematic representation of apparatus useful in this invention.

Figure 2 is a fragmentary perspective view showing filamentary material arrangement when first assembled into a loose batt.

Figure 3 is a similar fragmentary perspective view showing the appearance of the batt of Figure 2 after portions of some of the filamentary material have been forcibly oriented by needle-punching. The upper and lower (horizontal) surface areas of the needled batt of Figure 3 are slightly less than that of the loose batt of Figure 2, but the thickness of the batt of Figure 3 is slightly greater than the thickness of the batt of Figure 2. Forcible orientation of portions of the filamentary material results in contraction of the surface areas normal to the direction of needling of the batt and a slight increase in the thickness of the batt.

Figure 4 shows the appearance of a batt comprising retractable predominantly synthetic organic continuous filamentary material after some of the filamentary material has been first forcibly oriented by needle-punching and then treated to retract the filamentary material. The batt is substantially more compact than an unretracted batt, and the horizontal surface area of the needled, retracted batt is less than that of the batt prior to retraction. The thickness of the batt is usually slightly greater than the thickness of the unretracted batt.

Figure 5 shows a similar batt after forcible orientation of portions of some of the filamentary material, retraction and pressing. Pressing does not change substantially either the horizontal surface area or the batt strength.

In the apparatus shown in Figure 1, movable belt 11 supports filamentary material being processed according to this invention. Superimposed layers of filamentary material 12 are deposited on the belt by hand or mechanical means, as desired, for transport through needle loom 13 which reciprocates needles into and out of the loose layered batt of filamentary material, forcibly orienting portions of some of the filamentary components into at least one adjacent layer and preferably into a position substantially perpendicular to the faces of the batt. Needle-punching results in contraction of the surface areas of the batt normal to the direction of needling, and the needle-punched batt at 14 is shown to have smaller surface area than that of the loose layered batt prior to needling. The needle-punched batt at 14 may be used without further treatment and is highly useful in a number of applications. A needle-punched batt of predominantly retractable filamentary material optionally may be passed through oven 15 to further compact the batt and increase its density by retracting the filamentary material. Retraction of the batt as by heating to suitable temperature results in further reduction in the upper surface area of the batt, as shown at 16. Optionally, also a retracted or unretracted needle-punched batt may be pressed by passing through rolls 17 which forward the batt to a collection point. Roll pressure may be adjusted to compress the strip to slightly reduced thickness, if desired.

In general, the objects of the present invention are ac-

complished by forming a loose layered batt of predominantly synthetic organic continuous filamentary material, the layered batt having substantially parallel top and bottom faces with predominant orientation of the component filamentary material parallel to the faces of the batt, and forcibly orienting portions of some of the filamentary components into at least one adjacent layer of filamentary material, preferably into a position substantially perpendicular to the faces of the batt, to produce a coherent non-woven felt-like article of unbonded filamentary material. The invention extends to exposure of such articles, in which at least part of the component filamentary material is characterized by a capacity for retracting (that is, shortening, as by crimping or shrinking, upon being heated or otherwise suitably treated), to conditions effective to retract the retractable filamentary material, whereupon the batt becomes even more compact while remaining unbonded and felt-like. Thus, this invention contemplates as a principal product a non-woven coherent felt-like article of unbonded filamentary material containing a preponderance of synthetic organic continuous filamentary material, in which portions of some of the filamentary material are oriented in the thickness direction of the batt. The phrase "predominantly synthetic organic continuous filamentary material" as used herein refers to filamentary material more than 50% of which possesses essentially three properties, namely, it is synthetic, organic, and continuous in character.

Coherent non-woven unbonded felt-like articles may be prepared in accordance with this invention using all unretractable filaments but in accordance with a preferred embodiment part of the filamentary material used has the ability to retract when properly treated, as with heat or a swelling agent. The retraction may result from a simple reduction in length (that is, shrinking) or from a distortion of the filament into an irregular shape as by crimping or curling or both. The retractability or degree of retraction refers to a free filament at the treating conditions and is expressed conveniently as the percent decrease (based upon the original value) in shortest distance between two points on an individual filament; thus, when both shrinking and crimping occur, it is a summation of the effect produced by diminution in length and assumption of a more irregular path between the points of measurement. In some instances, it is desirable to prepare articles in accordance with this invention composed entirely of retractable filaments. Materials not retractable under the conditions of treatment can be blended with retractable synthetic filamentary material or layered with it in order to achieve special effects. Thus, glass filament which exhibits zero retractability and/or wool fibers which are essentially not retractable may be blended with a predominant proportion of synthetic organic continuous filaments.

All synthetic organic continuous filamentary material can be utilized in this invention and, where it is desired to produce a retracted product, practically all synthetic polymeric filament-forming compositions can be manufactured so as to have the necessary retractability. In addition to those exemplified hereinafter, these polymers include polyamides (e.g., polyhexamethylene adipamide, polyhexamethylene sebacamide, poly-epsilon-caproamide, and copolymers of these or other polyamides), polyesters (e.g., polyethylene terephthalate, polyethylene sebacate), polyesteramides, polyureas, polyurethanes, acrylonitrile polymers (including copolymers of acrylonitrile, especially with other ethylenically unsaturated monomers, such as vinyl chloride, vinyl acetate, methyl acrylate, and vinyl pyridine), vinyl polymers generally (e.g., polyvinyl acetate, polyvinyl chloride, and polystyrene), polymerized fluorolefins (e.g., polytetrafluoroethylene, polytrifluoromonomochloroethylene, polyhexafluoropropylene), polymerized hydrocarbons (e.g., polyethylene) and halogenated derivatives thereof, synthetic proteinaceous polymers, and

cellulosics (including esters, ethers, regenerated cellulose, and similar derivatives of cellulose). Silk and casein may also be used in minor amounts.

Continuous filamentary material useful in the present invention may be drawn off directly from a spinning (i.e., polymer extrusion) unit, usually as a bundle of identical filaments, or may be supplied from a package or other storage device for yarn already spun. The filamentary components may be formed into a layered batt manually or mechanically by feeding them onto a collecting surface where they accumulate in overlapping layers, the individual filamentary components in each layer being predominantly coplanar, lying parallel to the collecting surface and to the bottom and top of the batt so formed. Conveniently, the step of batt formation will be accomplished by mechanical means, such as forwarding jets, which may be operated to lay the filaments down at random or in some desired pattern. The collecting surface may be rotated or oscillated to promote even accumulation of the filaments; a moving belt used as the collecting surface also can convey the formed loose layered batt to the location where portions of some of the component filaments will be oriented forcibly to a position substantially perpendicular to the faces of the batt.

Depositing filaments with fluid jets permits formation of batts by elimination of blending procedures, and generally simplifies handling of starting materials. It also facilitates the use of continuous mono- or multifilaments, or continuous lengths of spun staple yarns in the preparation of the batt. Heretofore, use of continuous filaments in felt structures has been confined to woven backings or cores. Synthetic filaments are initially produced as continuous filaments, and use in this form simplifies the manufacturing operation. The use of continuous filaments imparts added compactness and strength to the product, which may range from a soft pliable to a hard stiff felt.

Regardless of how the batt is formed, or the type of continuous filamentary material used (e.g., bulked yarns, monofilament or multifilament yarns either twisted or untwisted, rope, tow, thread, ribbon, spun staple yarns, braid, etc.), the batt will ordinarily have been built up gradually by superposition of a number of layers of material. The resulting batt consists initially of a loose, fluffy mass in which filamentary components may be oriented in layers usually in planes parallel to the belt or other surface on which the batt is formed.

The linear azimuthal orientation of the layers of filaments in any loose batt may be random or may be predetermined to any azimuthal angle. Preferably, the filamentary components of adjacent layers lie at an azimuthal angle of between about 45° and 90° to one another and most preferably are oriented 90° from one another. Desirably, adjacent layers of filamentary components will have an average difference in azimuthal linear orientation of at least 5°. For example, a batt having random orientation will have an average difference of about 45° in azimuthal linear orientation between adjacent layers.

These filamentary components will remain oriented in layers more or less parallel to the faces of the final product unless some way is found to cause them to interlock between layers. A surprising feature of the present invention is the discovery that a coherent strong, pliable non-woven felt-like product having exceptional properties is obtained even when relatively small numbers of the filaments have been reoriented by needle-punching so that portions of the filaments are positioned in at least two layers of filaments.

The preferred method of achieving the required orientation of filaments in the batt is needle-punching, which is conveniently accomplished in a conventional needle loom. Such a loom has a large number of closely spaced parallel reciprocating needles designed to catch or drag filaments through the batt to interlock them.

mentary material as the needles move into the batt. Relative movement between the batt and the needling location may be either intermittent (while the needles are drawn clear of the batt) or continuous. To maintain the dimensional stability of the batt during needle-punching, it is usually advisable to feed simultaneously to the needle loom a supporting layer, for example, a layer such as a cheesecloth, a film, or a warp of the same fibers as in the batt. The supporting layer may be readily stripped after the punching operation, or if of the same fiber composition, may be retained in the punched batt. This type of loom is well known for use in textile operations, so further description is unnecessary. Of course, other suitable means may be used for forcibly orienting filaments into the desired position; for example, the batt may be hand-punched with an instrument effective to orient one or more filaments from the surface toward the interior of the batt, but such a procedure is quite tedious, of course.

Products formed by needle-punching loose batts according to this invention have many of the desirable characteristics of wool felts, despite structural dissimilarities observable upon close inspection. No difficulty is encountered in reaching and even exceeding in many cases customary felt densities in these articles. They are readily distinguishable from non-wool felt-like products containing thermoplastic filaments bonded by heat or adhesives to one another because of their superior pliability and higher split strength compared with the relatively stiff (nyielding) character and low split strength of bonded structures. In tensile strength, the products of the present invention compare very favorably with properties of conventional felts and felt-like products, including those made from synthetic staple fibers.

The rather fuzzy surface of the product can be smoothed by pressing. A heated pressing surface may induce retraction of surface filaments, but the temperature should be maintained below the softening temperature of the fiber to prevent fusion. This added compacting treatment is not essential in the majority of uses, nor need the product be subjected to any equivalent of fulling. The initial conditions of batt density and the intensity of treatment can be chosen to produce practically any desired density and coherence in the product without necessity for any rubbing pretreatment or fulling after-treatment.

The practice of this invention is exemplified below in some detail. In all the examples, physical characteristics of the articles mentioned were determined (unless otherwise indicated) according to recognized felt testing methods of the American Society for Testing Materials, specifically ASTM-D-461-53.

#### EXAMPLE I

Polyethylene terephthalate is melt-spun from flakes by the process described by Hebeler in Patent 2,604,689 into continuous filaments of 3 denier each. A conventional tow-forwarding jet passes a bundle of 20 filaments through an air diffuser, which opens up the bundle, then onto a cylindrical roll. The roll is rotated slowly and the multifilament yarn is traversed back and forth the width of the roll so that it winds in a helical configuration and the filaments in adjacent layers cross at an angle of at least about 5°. After several minutes, the winding is discontinued and the accumulation of yarn on the roll is removed by cutting along the surface of the roll parallel to the roll axis. This forms a layered non-woven loose batt of filaments. Batt length is equivalent to the circumference of the roll and width is about the same as the roll width. The batt is passed through a needle loom and needled alternately from the top and bottom for a total of 16 times (8 times per face of the batt). Each pass through the loom results in 120 needle penetrations per square inch of batt surface, a total of 1920 penetrations for the 16 passes. As a result of the nee-

dling, the face of the batt contracts and the thickness increases. Density (areal) of the felt is 32 oz./sq. yd. The product surfaces are quite smooth, showing only slight indentations produced by the needle-punching, and lacking any visible recurrent pattern of orientation of the component filaments in azimuth. No needle-formed channels are apparent. The product has a high tensile strength but is pliable enough to be bent easily by hand about a sharp corner without noticeable separation of filaments.

#### EXAMPLE II

Continuous multifilaments of crimpable polyethylene terephthalate retractable to the extent of at least about 15% are produced by extrusion through a 34-hole spinneret and drawing by an air jet to approximately 3 denier per filament as disclosed by Hebeler in Patent 2,604,689. The filaments are blown apart by the jet and deposited unrelaxed in a perforated basket until the random assemblage accumulates to a depth of 1.5 inches. The specific gravity of the batt-like mass is about 0.01. Needle-punching the batt with a needle loom equipped with regular barbed needles (15 x 18 x 25 x 3½) results in 50 needle penetrations per square inch of batt surface. After needle-punching once from the top of the batt, it is turned over and run through the needle loom again to punch it from the other side to give a specific gravity of about 0.11. The article so produced is a coherent non-woven pliable felt-like product, suitable as a filter, of smaller face-surface area and slightly greater thickness than the batt prior to needling.

Immersion of the batt in boiling water for 2 minutes results in further retraction of the filaments and reduction of the area of the batt by about 25%, producing an even more compact felt-like mass. Upon tensile testing (Instron) of a 2-inch strip of the retracted product, a force of about 40 pounds is required to break it, corresponding to about 265 lbs./sq. in., at breaking elongation of slightly over 100%. The same force is necessary to break a similar strip taken transversely to the one just tested. This article is particularly useful as a filter for liquids.

In the following examples the batts were prepared from continuous multifilaments collected onto a moving belt in overlapping layers in each of which the filaments were oriented at 45° to the direction of belt movement, being oriented at a right angle to one another in alternate layers. This can be accomplished by means of delivery jets oscillating diagonally to the belt; however, the apparatus actually used comprised a rotating hollow shaft through which the yarn was passed and delivered onto two vertical screws that supported the yarn in an elongated oval and then dropped it on the belt, being the apparatus shown in Figure 10 of a patent application filed by D. S. Adams and J. F. Bowling on September 10, 1954, as Serial No. 455,192, and described in their specification.

#### EXAMPLE III

A batt 30 inches wide is constructed from 400 denier, 60 filament yarn composed of polytetrafluoroethylene on a moving belt with the filaments in alternate layers oriented at a linear azimuthal angle of about 90° along diagonals of the belt as just described. The batt is punched twice on a standard plate-type needle loom (Hunter Machine Company) using regular barbed needles (15 x 18 x 25 x 3½) so that the batt receives 120 penetrations per square inch during each pass through the loom. The batt is folded double and punched 5 additional times under the same conditions, alternately from each side. The batt then is doubled again and punched an additional 15 times, alternately from each side, with the same punching frequency as before. The batt contracted about 13% during the needling and was converted to a felt-like product weighing 7.3 lbs./sq. yd. which is useful as a filter for liquids,

especially corrosive fluids to which ordinary filter cloths are not resistant.

Duplication of the above procedure with highly drawn (7 times) polytetrafluoroethylene filaments produces a similar felt-like article that can be compacted further, by heating to a temperature of about 300° C., to produce a retracted but still unbonded pliable felt-like article. This product is particularly useful as a filter or as a sealing gasket.

#### EXAMPLE IV

A batt of continuous nylon (polyhexamethylene adipamide) multifilament of 840 total denier and 140 filaments with layer orientation as in Example III is punched 3 times from the same side to give a total needling frequency of 90 penetrations per square inch. The needled batt is plied 3 times and punched once from each side at a needling frequency of 120 penetrations per square inch during each pass. The 3-ply structure is then tripled again to a total thickness of 9 plies and punched 10 additional times, alternately from each side at a needling frequency of 120 penetrations per square inch during each pass. A coherent felt-like article useful as a polishing felt for glass results, having a density slightly in excess of the values for an SAE F-1 wool felt and a retracted needle-punched synthetic staple felt but with strength greatly superior to both, as indicated in the following table. The nylon felt is hard and relatively stiff.

Table I

| Felt                                    | Density<br>(g./cc.) | Weight<br>(lb./sq.<br>yd.) | Strength                      |                                                          |
|-----------------------------------------|---------------------|----------------------------|-------------------------------|----------------------------------------------------------|
|                                         |                     |                            | Split<br>(lb./2 in.<br>width) | Tensile <sup>1</sup><br>(lb./in.<br>per lb./<br>sq. yd.) |
| Example IV                              | .43                 | 7.6                        | 48                            | 190                                                      |
| Polyethylene terephthalate<br>retracted | .37                 | 6.4                        | 45                            | 99.3                                                     |
| SAE F-1 wool                            | .34                 | 7.6                        | 33                            | 31.3                                                     |

<sup>1</sup> Tensile strength was measured according to A.S.T.M. procedures and the data adjusted to account for differences in density, etc., in order to provide an accurate comparison between felts.

Table I shows that under comparable conditions articles produced from continuous filaments according to the present invention have properties superior to wool felts or synthetic felt-like articles formed from needle-punched staple batts (even though retracted).

#### EXAMPLE V

Following the procedure of the above two examples, a batt with linear azimuthal orientation of the filaments of about 90° difference between layers is constructed from high-tenacity rayon yarn ("Super Cordura") having a total denier of 1650, with 720 filaments. With the needle loam and barbed needles of Example III this batt is punched three times from one side at a needling frequency of 30 penetrations per square inch during each pass. The batt is tripled by laying up three plies and punched for an additional 8 passes, alternately from each side, receiving 120 penetrations per square inch during each pass. The batt contracted about 12% during the needling, resulting in a felt-like article weighing 18 oz./sq. yd., and useful as a reinforcement for rubber in conveyor belts.

The expensive and time-consuming steps of hardening and fulling wool fibers are completely eliminated by this invention, and the retraction step required to render staple batts felt-like is rendered unnecessary. The steps of crimping synthetic staple and carding synthetic staple or wool also are obviated. Retraction is an optional final step in the practice of the present invention; with some materials (e.g., nylon) retraction treatment adversely affects desirable characteristics of toughness and

abrasion resistance, as by decreasing molecular orientation of the filaments.

The compactness and strength of the products of this invention are not dependent upon interfiber adhesion or softening and partial fusion. In fact, such fusion is undesirable because of its adverse effect upon physical characteristics of the product. For light-weight materials where a high initial degree of interlocking is desired, the starting material itself may be crimped, a distortion usually not lost and occasionally even enhanced by the subsequent retraction by treatment with heat or a swelling agent. The original degree of molecular orientation, usually largely the result of drawing, may be adjusted for a given use, with due regard to the desired resulting fiber elongation and tenacity and the influence of draw ratio upon retractability of the particular synthetic filamentary material used.

Felt-like materials of substantially any desired characteristics may be formed according to this invention. Thus, rather than the type of product determining utility, as so often happens, here the products of the invention may be made so as to fill a wide variety of uses for non-woven materials. These felt-like materials may be manufactured in suitable form for use as wet and dry felts; filter media, carpets and their underliners, insulation, sound absorbents, chemical-resistant work clothes, and many other industrial and apparel uses. The transverse and longitudinal properties may be made practically identical by blending or layering, or wide differences between them may be secured by sufficient orientation of the starting filaments or fibers. The shape of the product may be determined by placing the batt against or around a fixed form so that the batt assumes the configuration of the form during retraction, and pressing may be used to improve shape correspondence in this process modification.

Any synthetic organic continuous filamentary material is suitable for use in the practice of this invention. By "continuous," as used herein, is meant any length greater than about eight inches. Preferably, continuous filaments having an average length greater than about eight inches are employed because needling of a loose batt of predominantly synthetic organic filamentary material having an average length of at least about eight inches results in contraction of the batt, thereby producing a strong coherent felt-like product without recourse to retracting the batt. Thus, merely needle-punching a loose batt of continuous filamentary material in accordance with this invention without chemical or heat treatment decreases the surface area of the batt as contrasted with an increase in surface area when a loose batt of conventional staple fibers is needle-punched. If desired, blends with animal, vegetable, or mineral continuous filamentary material may be employed although it is preferred to utilize synthetic organic continuous filaments alone. Of course, more than one kind of filament may be blended or layered together. It will be appreciated that needling of a batt of continuous filaments will result in breaking of some filaments and that the product produced may contain a considerable number of broken filaments depending upon the amount of needling. In all cases, however, the product will contain predominantly continuous filaments, and these filaments will be synthetic and organic in character.

Most synthetic organic continuous filaments can be produced in retractable form for use according to a preferred embodiment of this invention in which additional compactness is induced by retracting the filaments after needling. As suggested, the retraction treatment may consist of heating by various means, as by application of water, oil, steam, air or other fluid which is relatively inert with respect to the particular filamentary material or it may involve exposure of the material to a swelling agent in addition to or in place of the heat treatment. A combination of chemical and physical

treatments may be used, mild acid and alkali baths being examples of what often may be acceptable chemical treatments. Any method of shortening the end-to-end length of the filamentary material without too adversely affecting filament properties and fibrous structure is acceptable. If the filaments are to be retracted in a liquid bath, instead of by heating, a conveyor belt may be arranged to carry the batt through a tank where the filaments are submerged in or sprayed with the retraction-inducing liquid. This may be followed by suitable means for removing the liquid, such as wringer rolls and a drier, or by extraction, as will be understood in the art. The time of treatment may vary from a few seconds to hours, although for simplicity, times of the order of a minute or so are preferred. Either retracted or unretracted products of this invention can be pressed for smoothing of the surface or additional compaction of the filaments, if desired. Where a retracted batt is desired, it is preferred that the filamentary material utilized be retractable in length to the extent of at least about 15% in order to achieve substantial benefits from the retraction step.

In addition to the uses mentioned above for the products of this invention may be mentioned body armor and flak curtains, shaft packing, reinforced plastics, laminates, polishing felts, grease seals, wicking felts, mechanical felts, wet and dry papermakers' felts, apparel felts, artificial leather, sanforizing blankets, tire cord fabrics, steaming pads, roll covers, and shock and vibration mountings. Many other suitable uses for these products will become apparent to anyone undertaking to practice the present invention.

In general, the continuous filament needled, unretracted felt-like articles of this invention possess superior abrasion resistance, chemical resistance, thermal stability, and tenacity to felt-like articles made from staple fibers.

This application is a continuation-in-part of application Serial Number 312,067, filed September 29, 1952, now abandoned, by Herbert G. Lauterbach and Harry M. Norton, and application Serial Number 436,014, filed June 11, 1954 by Herbert G. Lauterbach.

The claimed invention:

1. A non-woven coherent felt-like article comprising predominantly synthetic organic continuous filamentary material characterized by predominantly coplanar superimposed layers of the filamentary components, the filaments in each layer being oriented at an angle relative to adjacent filaments in adjacent layers, with portions of some of the filamentary components from each layer oriented into at least one adjacent layer.

2. The product of claim 1 in which the continuous filamentary components are at least partly retractable to diminished length.

3. The product of claim 1 in which the filamentary material is a polyamide.

4. The product of claim 1 in which the filamentary material is rayon.

5. The product of claim 1 in which the filamentary material is a polyester.

6. The product of claim 1 in which the filamentary material is polytetrafluoroethylene.

7. A non-woven retracted coherent felt-like article

comprising predominantly synthetic organic continuous filamentary material characterized by predominantly coplanar superimposed layers of the filamentary components, the filaments in each layer being oriented at an angle relative to adjacent filaments in adjacent layers, with portions of some of the filamentary components from each layer oriented into at least one adjacent layer.

8. The product of claim 7 in which the filamentary material is polyethylene terephthalate.

9. The product of claim 7 in which the filamentary material is polytetrafluoroethylene.

10. The product of claim 7 in which the filamentary material is a polyamide.

11. A process for preparing a non-woven coherent felt-like article comprising forming a loose batt of predominantly synthetic organic continuous filamentary material as a plurality of superimposed substantially parallel layers, the filaments in each layer being oriented at an angle relative to adjacent filaments in adjacent layers, and forcibly orienting portions of some of the filamentary components into at least one adjacent layer.

12. The process of claim 11 in which substantially all of the continuous filamentary material is retractable.

13. The process of claim 12 in which the felt-like article produced is retracted.

14. The process of claim 12 in which the filamentary material is polyethylene terephthalate.

15. The process of claim 12 in which the filamentary material is polytetrafluoroethylene.

16. The process of claim 12 in which the filamentary material is polyhexamethylene adipamide.

17. The process for preparing a felt-like product which comprises forming a mass of heat retractable continuous synthetic filaments into a loose batt, said filaments being retractable by at least 15% in length when heated below the fusion temperature, punching portions of some of the filaments into the batt in a direction substantially perpendicular to the faces of the batt, and then without other treatment heating the filaments so that they retract at least 15% in length and remain free to move over each other though under frictional constraint from mutual contact until they retract sufficiently to compact the batt to a felt-like product.

18. The process for preparing a felt-like product which comprises forming a mass of heat retractable substantially continuous polyethylene terephthalate filaments into a loose batt, said filaments being retractable by at least 15% in length when heated below the fusion temperature, punching some of the filaments for part of their length into the batt in a direction substantially perpendicular to the faces of the batt, and then without other treatment heating the filaments below the fusion temperature to cause them to retract at least 15% in length without adhering with resulting compaction of the batt to a felt-like product.

#### References Cited in the file of this patent

#### UNITED STATES PATENTS

|           |              |               |
|-----------|--------------|---------------|
| 2,181,043 | Boeddinghaus | Nov. 21, 1939 |
| 2,336,797 | Maxwell      | Dec. 14, 1943 |
| 2,416,390 | Hitt         | Feb. 25, 1947 |
| 2,437,689 | Francis      | Mar. 16, 1948 |